

No. 852,612.

PATENTED MAY 7, 1907.

W. G. PERKINS.

PROCESS OF DESULFURIZING AND SUBSEQUENT SMELTING.

APPLICATION FILED JAN. 22, 1906.



Attest  
C. S. Madsen  
Edward N. Barton

Inventor:  
Walter G. Perkins  
By Spear & Sally Atty

# UNITED STATES PATENT OFFICE.

WALTER G. PERKINS, OF SAN FRANCISCO, CALIFORNIA.

## PROCESS OF DESULFURIZING AND SUBSEQUENT SMELTING.

No. 852,612.

Specification of Letters Patent.

Patented May 7, 1907.

Application filed January 22, 1906. Serial No. 297,354.

*To all whom it may concern:*

Be it known that I, WALTER G. PERKINS, a subject of the King of Great Britain, residing at San Francisco, in the county of San Francisco and State of California, have invented certain new and useful Improvements in Processes of Desulfurization and Subsequent Smelting, of which the following is a specification.

10 This invention relates to the treatment of metalliferous substances and chemical compounds by heat, and more particularly to a process of desulfurizing, or roasting, and smelting ores, concentrates, matte, or any 15 other mineral or chemical substance in one continuous operation by means of a liquid or gaseous fuel, together with the combustible material in the ore itself.

The present invention is particularly 20 adapted to the smelting of pyritic ore in a finely divided state, and concentrates such as are the products of the various concentrating tables, a large percentage of which may pass a screen of 200 mesh to the inch. Material 25 such as this is extremely difficult to treat even by the universally used method of first desulfurizing in any of the turret or reverberatory roasting furnace and then smelting the calcined material in a reverberatory 30 smelting furnace, making two stages of the process and consequently the handling of the material a second time, which entails losses in values and extra expense. During the roasting process there are large losses in the 35 form of flue dust caused by the air current going through the furnace and taking with it a large percentage of the finely divided material which has to be collected in large dust settling chambers at almost a prohibitive expense; this will be almost entirely averted 40 by my process because there will always be a high column or volume of charge above the twyer zone where the air enters and where the desulfurization is taking place. The actual smelting operation does not take place 45 in this receptacle, but merely the desulfurizing, the charge descending to the throat of the lower receptacle before becoming thoroughly fused and in a sufficiently molten 50 form for the matte to separate from the slag.

The drawing submitted embodying a form of apparatus capable of carrying out the process described is in accordance with the examiner's requirement.

55 In this drawing Figure 1 is a vertical section; Fig. 2 is a longitudinal view of a por-

tion of the furnace taken at right angles to Fig. 1.

In the drawing 1 indicates the stack or main portion of the furnace, which may be 60 of the usual size and style, and around which is arranged a wind-box 2 which communicates with the interior of the stack through twyers or passages 3. Beneath the stack is a hollow crucible, which is preferably removable, and which is adapted to be separately heated by gaseous or atomized fuel introduced directly into it. The crucible is contracted at the top so as to form a throat in which the actual smelting operation takes place. It will therefore be understood that the gaseous or other fuel is introduced into the hollow crucible independently of the smelting zone and is allowed and permitted to expand and attain a full combustion, 70 which it could not if introduced directly into a mass of finely divided material. In such a case, the gaseous fuel, having no opportunity to expand and to receive the necessary oxygen for perfect combustion, will simply back out and become inert. When the individual pieces of material are of comparatively large size, interstices between the members of the mass, may permit the expansion and combustion of a gaseous or atomized fuel; but such a fuel introduced directly 75 into a mass of very finely divided material, cannot do effective work for the reasons before stated. But with my process the steps are continuous; whereby the heat is 80 conserved and utilized, and the movement of the material is automatic and by gravity, which reduces the cost of handling and treatment to the minimum. Another advantage arising from my process is the ease with which 85 the temperature can be controlled, in contradistinction to the non-fuel pyritic or the added solid fuel of the semi-pyritic smelting processes, thereby making it possible to treat extremely refractory ores which require temperatures higher than can be obtained in pyritic or semi-pyritic smelting, because if more air is supplied to a pyritic smelting furnace 90 than can combine with the elements it will decrease the temperature of the mass and cause the furnace to become cold or "freeze," and if solid fuel be fed to the furnace with the ore, as in semi-pyritic smelting, there is danger of the temperature of the mass rising 95 above the smelting zone to such a degree as to cause "overfire" of the top of the material in furnace and lowering of the temperature at 100

105 110

the bottom or smelting zone, which causes a furnace to run badly. Furthermore, by not having a quantity of carbonaceous solid fuel mixed with the material to be smelted, ; the air blown into the charge through the twy whole or wind box is used entirely for oxidizing the elements in the charge and is not consumed by the carbon of the solid fuel to generate heat for carrying on the operation, 10 as in semi-pyritic smelting. The foreign heat being supplied by gas or oil with an air blast of its own, would give practically a neutral atmosphere, as in reverberatory furnace smelting, and would, after expending itself 15 on the smelting, render the excess available to ascend into the charge above to supply the requisite heat to carry on the chemical reaction between the elements in the charge and the air supplied through the twy whole. It also 20 has the advantage of keeping the smelting zone at one point in the furnace shaft, thereby preventing the danger of "overfire," which cannot be controlled when solid carbonaceous fuel is mixed with the charge, as 25 the point of fusion rises and lowers according to the condition of the furnace and causes most of the evils encountered in blast furnace smelting. Besides being able to control the heat when supplied from gas or oil it is more 30 economical and also avoids the introduction of foreign substances into the charge in the form of ash, etc., which would add just that much more to the dross from which the values must be separated. Still another advan- 35 tage is that a smelter can be operated at a point removed from transportation by the generation of producer gas from wood, thereby rendering the smelter independent of a coal or coke supply, and there are very few 40 points where either coal, oil or wood cannot be obtained, either being used for making producer gas.

In carrying out my process, the material to be roasted and smelted is fed into a receptacle having places in its sides, as a twy whole or wind box, preferably near the bottom, for the admission of air, and an opening in the bottom for the escape of the material after it has been initially treated or desulfurized. A 45 second receptacle is arranged directly below the first one into which said material falls by gravity after it has become semi-fused or liquefied and in which the separation of the more valuable material from the slag takes 50 place.

Means are provided for heating the mass to such a degree of temperature as will permit the combustible portions of the mass, as the sulfur, etc., to combine chemically with 55 the oxygen of the air which is introduced through the twy whole in the sides of the mass and caused to pass upward therethrough. In this manner, after the combustion by decomposition of the sulfids has commenced, 60 the heat from the mass, together with that

from the applied smelting heat in the lower receptacle, will be sufficient to purify or desulfurize the mass for further or final treatment.

As the mass becomes heated and semi-fused it will project down through the opening in the bottom of the upper receptacle into the lower receptacle, where it will be subjected to a degree of heat sufficient to completely fuse or melt it and cause it to fall 70 into the lower receptacle where the valuable portions as matte, or metal, which being heavier than the dross or slag, will settle in the bottom and from whence it can be removed in the ordinary manner, as by continuous overflow, etc.

The heat from external sources is preferably obtained from an inflammable gas, or from fluid fuel as oil reduced to a gaseous form in any well known manner, and it is 85 applied entirely through the lower receptacle. When the process is originally started, the lower receptacle will be empty, and the heat will pass through the opening in the bottom of the upper receptacle, into and up 90 through the mass of material therein until it becomes hot enough to cause the sulfur to burn and be eliminated therefrom. When the mass reaches such a degree of temperature, air is admitted through the twy whole in 95 the sides of the receptacle which will support the combustion of the sulfur and cause a partial fusion of the less easily fused portions. This semi-fused mass will then settle down 100 to the bottom of the receptacle and partly protrude through the opening in the bottom thereof into the lower receptacle where it will be subjected to the full effect of the applied heat therein which will cause it to be 105 completely fused or melted and drop through the opening into the lower receptacle. As the lower portion of the mass in the upper receptacle is thus melted and falls away, more of the mass will take its place and protrude and in turn will be melted and fall 110 away, thereby causing the process to be continuous.

From the foregoing it will be seen that as the material is fed in at the top of the upper receptacle it gradually becomes heated as it passes downward, then ignites and assists in supplying the necessary heat to desulfurize or purify itself, and finally it passes down into the lower receptacle where it is completely smelted and the valuable portions separated from the slag. The heat from the desulfurizing process is utilized, also the heat from the gaseous fuel, because it has to pass up through the entire mass to find an 120 exit, making it economical and quick to treat the material in a continuous process. The material to be treated may be in any form, as 125 ores, concentrates, matte, etc., and is preferably fed in at the top, and the propor- 130

tions of sulfur, or other combustible substance, may vary within wide limits, and by controlling the admission of air through the twyers and gaseous fuel through the lower receptacle the process can be carried on successfully and continuously.

When it is desired to heat the air that is being introduced into the mass through the twyers or wind box, an excess of heat may be generated at the bottom and a portion of it can be transferred to the wind box by a valved conduit or by-pass where it will be commingled with the ingoing air and thereby heat the same. In this manner the heating of the mass can be controlled either at the bottom or through the wind box, or both, and thus secure the most desirable results with different kinds of ores or substances.

Having described my invention, what I claim as new and desire to secure by Letters 20 Patent, is:

The process of treating ores in a finely divided state which consists in introducing gaseous fuel into a heated space below the smelting zone and then passing said fuel 25 mixed with air up through the smelting zone and at the same time introducing air into the smelting zone.

In testimony whereof I have affixed my signature, in presence of two witnesses, this 30 15th day of January, 1906.

WALTER G. PERKINS.

Witnesses:

M. R. SEELY,  
F. M. BARTER.